

Nov. 10, 1925.

1,560,941

H. C. MILLER

ORNAMENTED SURFACE AND METHOD OF FORMING THE SAME

Filed July 13, 1925

*Fig. 2.*



*Fig. 1.*



3

*Fig. 3.*



Inventor

*Herman C. Miller.*

By *Frease & Bond*

Attorneys

## UNITED STATES PATENT OFFICE.

HERMAN C. MILLER, OF CANTON, OHIO, ASSIGNOR TO THE UNITED METAL PRODUCTS COMPANY, OF CANTON, OHIO, A CORPORATION OF OHIO.

## ORNAMENTED SURFACE AND METHOD OF FORMING THE SAME.

Application filed July 13, 1925. Serial No. 43,214.

*To all whom it may concern:*

Be it known that I, HERMAN C. MILLER, a citizen of the United States, residing at Canton, in the county of Stark and State 5 of Ohio, have invented certain new and useful Improvements in Ornamented Surfaces and Methods of Forming the Same, of which the following is a specification.

This invention relates to ornamenting surfaces 10 of sheet metal, tile, wood, glass or similar material, and more particularly to a novel method of ornamenting the surfaces of sheet metal doors, sashes, baseboards and the like.

15 It is well known that sheet metal has to a large extent replaced wood for use in doors, sashes, baseboards and other building materials, particularly in the construction of office buildings and similar large 20 edifices. It is customary to paint or enamel such metal material in imitation of wood grain, thus giving the higher priced and more durable metal structure the appearance of the ordinary wooden doors, sashes and 25 the like.

The object of the present invention is to provide an ornamental surface for sheet metal and the like in which any desired design or effect may be carried out, the finished 30 surface having irregular ribs and valleys, the whole giving the impression of a metallic finish rather than the usual wood finish.

An embodiment of the invention is illustrated in the accompanying drawing, in 35 which—

Figure 1 is an elevation of a portion of the surface ornamented by the improved method;

Fig. 2, a section through a sheet of metal 40 with the finish coating thereon before the high spots in the surface have been smoothed or cut; and

Fig. 3, a similar view of the finished surface.

45 Similar numerals refer to corresponding parts throughout the several figures of the drawing.

In carrying out the invention to ornament the surface of a metal sheet as shown 50 at 1, a rust proof metal primer is first applied to the surface of the metal which is to be ornamented.

A composition which may contain red

lead, whiting, oil, varnish and other ingredients mixed into a paste, is then applied 55 to the surface of the sheet with a knife or trowel and worked into any desired design or configuration with brushes or suitable tools.

This composition is indicated by the numeral 2 and in cross section may assume a configuration similar to that shown in Fig. 2, having alternate irregular valleys 3 and ribs 4.

The sheet is then placed in an oven and 60 kiln and baked until the coating becomes extremely hard, after which the top surfaces of the ribs 4 are ground or filed forming the flat irregular surfaces 5, as shown in Figs. 1 and 3.

70 The decorated surfaces may then be painted in any desired manner. It has been found by experience that very artistic results may be obtained by painting the entire surface with bronze, gold or silver paint, and 75 after the same has dried a coat of green or other color is applied to the surface, and while wet the flat surfaces 5 are wiped off, leaving the gold bronze or silver thereon, while the valleys remain green. A coat of 80 varnish may be applied to the coated surface, after the same has thoroughly dried.

85 Although only one design of an ornamentation is illustrated, it has been found with experience that by the use of various instruments or tools, a great number of artistic finishes may be easily and quickly formed upon the coated surface, giving the impression of metal, rather than the usual wood finishes now in common use.

90 Although this finish is primarily intended for sheet metal doors, sashes, baseboards and the like, it is adaptable for use for ornamenting any surface, such as wood, tile, glass or other materials, it being understood 95 that where wood or similar materials is used the coating is sun dried instead of being baked in the furnace.

I claim:

1. The ornamenting process which consists in applying a plastic coating to a surface to be ornamented, forming ribs and valleys in said coating, hardening the coating and cutting away the high points of the ribs.

100 2. The ornamenting process which consists in applying a plastic coating to a sur-

face to be ornamented, forming ribs and valleys in said coating, hardening the coating and cutting away the high points of the ribs, forming flat surfaces in substantially 5 the same plane.

3. The ornamenting process which consists in applying a plastic coating to the surface of an article to be ornamented, forming ribs and valleys in said coating, baking the 10 coated article until the coating is hard and cutting away the high points of the ribs.

4. The ornamenting process which consists in applying a plastic coating to the surface of an article to be ornamented, forming 15 ribs and valleys in said coating, baking the coated article until the coating is hard and cutting away the high points of the ribs forming flat surfaces in substantially the same plane.

20 5. The ornamenting process which consists in applying a plastic coating to a surface to be ornamented, forming ribs and valleys in said coating, hardening the coating and cutting away the high points of the 25 ribs forming flat surfaces in substantially the same plane, painting the coated surface and permitting the paint to dry, painting the surface with a different color of paint

and wiping the second coat of paint from said flat surfaces while the paint is wet. 30

6. The ornamenting process which consists in applying a plastic coating to a surface to be ornamented, forming ribs and valleys in said coating, hardening the coating and cutting away the high points of the ribs 35 forming flat surfaces in substantially the same plane, painting the coated surface and permitting the paint to dry, painting the surface with a different color of paint and wiping the second coat of paint from said 40 flat surfaces while the paint is wet and covering said painted surface with a transparent water proof coating.

7. The ornamenting process which consists in applying a plastic coating to a surface to be ornamented, forming ribs and valleys in said coating, hardening the coating and cutting away the high points of the ribs, forming flat surfaces in substantially 50 the same plane, painting said ornamented surface and covering the painted surfaces with a transparent water proof covering.

In testimony that I claim the above, I have hereunto subscribed my name.

HERMAN C. MILLER.